

# UNITED STATES PATENT OFFICE.

WILLIAM A. SCHEUCH, OF NEW YORK, N. Y., ASSIGNOR TO WESTERN ELECTRIC COMPANY, INCORPORATED, OF NEW YORK, N. Y., A CORPORATION OF NEW YORK.

## ELECTRIC-RESISTANCE ALLOY.

1,337,276.

Specification of Letters Patent. Patented Apr. 20, 1920.

No Drawing.

Application filed August 3, 1917. Serial No. 184,229.

To all whom it may concern:

Be it known that I, WILLIAM A. SCHEUCH, a citizen of the United States, residing at New York, in the county of Bronx and State 5 of New York, have invented certain new and useful Improvements in Electric-Resistance Alloys, of which the following is a full, clear, concise, and exact description.

This invention relates to high resistance 10 alloys, and its object is to provide an alloy having a high specific resistance which possesses the properties essential to a high resistance element, such as durability and a melting point higher than that of pure 15 copper.

It is known that an alloy consisting of nickel and cobalt only, has a resistance somewhat greater than that of copper and that the specific resistance is quite appreciable 20 for compositions, ranging as much as from 60 to 95% of nickel and 40 to 5% of cobalt. The highest specific resistance for the two elements, namely, about eight times that of copper, is obtained with a composition 25 of approximately 80 to 85% of nickel and 20 to 15% of cobalt.

However, in accordance with this invention, it has been found that the specific resistance of a base alloy of nickel and cobalt 30 may be enormously increased by the addition of the metal titanium. Thus, an addition of 5% of titanium to the preferred base alloy of 80 to 85% of nickel and 20 to 15% of cobalt increases the resistance to approximately 35 forty times that of copper; while the addition of 7.5% of titanium increases the resistance to approximately fifty-six times that of copper. The addition of 20% of titanium, however, makes the alloy too brittle 40 to be readily worked and drawn at the present stage of the knowledge of working metals. It is, therefore, desirable that the titanium added should be less than 20%; and the preferred alloy is obtained by adding 45 approximately 10% titanium to a base alloy of 83% nickel and 17% cobalt, which would mean a mixture of approximately 75% nickel, 15% cobalt and 10% titanium.

Such an alloy, as cast, has the very high 50 specific resistance of more than 50 times that of copper and is malleable and very durable so that it has many important uses

in connection with electrical apparatus of various kinds.

Although it is preferred that the base 55 alloy should have a composition within the range of approximately 60 to 95% nickel and 40 to 5% cobalt, this invention is not limited to such a range, as an alloy having a fairly high specific resistance may be obtained by having the nickel content as low 60 as 40%.

It has also been found that this alloy of nickel, cobalt and titanium may have its working qualities considerably improved 65 and may be more readily melted by the addition thereto of small amounts of the metals, copper or manganese, or both. In general, it will not be found necessary to add more than 10% of either of the metals, copper or 70 manganese, or more than a 20% mixture of the two. Thus, an alloy containing 70% nickel, 14% cobalt, 8% titanium and 8% of either copper, manganese or a mixture of both, has been found quite satisfactory as 75 a high resistance element. It is to be understood, however, that this invention is not limited to an alloy containing copper and manganese, since these two metals may be omitted, if desired. 80

What is claimed is:

1. An alloy containing nickel,  $1\frac{1}{2}$  per cent. cobalt or more and titanium, the nickel being in excess of 50%. 85
2. A resistance element containing nickel,  $1\frac{1}{2}$  per cent. cobalt or more and titanium in substantial amounts.
3. A resistance element comprising nickel,  $1\frac{1}{2}$  per cent. cobalt or more and titanium, the titanium content being less than 20%. 90
4. A resistance element comprising nickel,  $1\frac{1}{2}$  per cent. cobalt or more and titanium, the titanium content being less than 12%.
5. A resistance element comprising nickel,  $1\frac{1}{2}$  per cent. cobalt or more and titanium, the nickel being in excess of 50%. 95
6. A resistance element comprising nickel,  $1\frac{1}{2}$  per cent. cobalt or more and titanium, the cobalt being less than 40% of the mixture.
7. A resistance element comprising 60 to 85% of nickel, 30 to 10% of cobalt, and titanium in a substantial amount. 100
8. A resistance element, approximately

- 90% of which is made up of nickel,  $1\frac{1}{2}$  per cent. cobalt or more and titanium.
9. An alloy comprising nickel,  $1\frac{1}{2}$  per cent. cobalt or more, titanium, and one or more metals having the properties of copper and manganese.
10. A resistance element comprising nickel,  $1\frac{1}{2}$  per cent. cobalt or more, titanium and manganese.
11. A resistance element comprising nickel,  $1\frac{1}{2}$  per cent. cobalt or more, titanium and copper.
12. A resistance element comprising nickel,  $1\frac{1}{2}$  per cent. cobalt or more, titanium, and substantial amounts of manganese and copper.
13. A resistance element comprising nickel,  $1\frac{1}{2}$  per cent. cobalt or more, titanium and manganese, the manganese content being less than 20%.
14. A resistance element comprising nickel,  $1\frac{1}{2}$  per cent. cobalt or more, titanium, and one or more metals having the properties of copper and manganese, said one or more metals being present in an amount less than 20%.
15. A resistance element comprising approximately 60 to 85% nickel, 10 to 30% cobalt, and titanium and one or more metals having the properties of manganese and copper.
16. A resistance element comprising approximately 70% nickel, 14% cobalt, 8%
- titanium, and 8% of one or more metals having the properties of copper and manganese.
17. A resistance element comprising approximately 70% nickel, 14% cobalt, 8% titanium, and 8% of manganese and copper.
18. An alloy comprising nickel,  $1\frac{1}{2}$  per cent. cobalt or more and titanium, said alloy being characterized by having a specific resistance greater than an alloy of the first two named ingredients.
19. An alloy comprising nickel,  $1\frac{1}{2}$  per cent. cobalt or more, titanium and manganese, the content of nickel being not less than 50% by weight of the whole, said alloy being characterized by having a specific resistance greater than an alloy of the first two named ingredients.
20. An alloy comprising nickel,  $1\frac{1}{2}$  per cent. cobalt or more, titanium and copper, the content of nickel being not less than 50% by weight of the whole, said alloy being characterized by having a specific resistance greater than an alloy of the first two named ingredients.
21. An alloy containing approximately 60 to 85% nickel, 10 to 30% cobalt, and titanium and one or more metals having the properties of manganese and copper.

In witness whereof I hereunto subscribe my name this 2nd day of August, A. D. 1917.

WILLIAM A. SCHEUCH.